

Sept. 27, 1949.

P. G. CHACE

2,482,899

CORROSION-RESISTING COMPOSITE METAL

Original Filed June 23, 1941



Paul G. Chace  
Inventor  
Haynes and Koenig  
Attorneys

## UNITED STATES PATENT OFFICE

2,482,899

CORROSION-RESISTING COMPOSITE  
METAL

Paul G. Chace, Attleboro Falls, Mass., assignor to  
Metals and Controls Corporation, Attleboro,  
Mass., a corporation of Massachusetts

Original application June 23, 1941, Serial No.  
399,398, now Patent No. 2,366,178, dated Janu-  
ary 2, 1945. Divided and this application No-  
vember 11, 1944, Serial No. 563,015

5 Claims. (Cl. 29—195.5)

1

This invention relates to composite metal ele-  
ments and particularly to bimetallic elements  
which are corrosion-resisting.

This application is a division of my co-pending  
application, Serial No. 399,398, filed June 23, 1941,  
Patent 2,366,178.

Among the several objects of the present in-  
vention are the provision of a composite thermo-  
static metal which is corrosion-resisting, which  
has an improved bond, and which has a long life  
when operating in corrosion-promoting atmos-  
pheres and mediums; the provision of composite  
thermostatic metal of the class described which  
has both good hot-rolling and good cold-rolling  
properties; and the provision of composite  
thermostatic metal of the type indicated which is  
relatively simple and economical to manufacture.  
Other objects will be in part obvious and in part  
pointed out hereinafter.

The invention accordingly comprises the in-  
gredients and combinations of ingredients, the  
proportions thereof, and features of composition,  
which will be exemplified in the products herein-  
after described, and the scope of the application  
of which will be indicated in the following claims.

In the accompanying drawing in which is illus-  
trated one of various possible embodiments of the  
invention, the single figure is a representation of  
a bimetallic element showing a strip of iron  
chromium alloy fused throughout its length to a  
similar strip of copper silicon alloy.

Many of the thermostatic elements commonly  
in use are subject to corrosion when used in the  
presence of moisture in places such as steam  
radiators, or water mixing valves, or in other in-  
stallations where corrosion-promoting fluids or  
atmospheres come in contact with the thermo-  
static metal. As a result, such elements fre-  
quently need replacing, and inasmuch as cor-  
rosion tends to reduce their activity and life, such  
corrosion may set up, unknown to the user,  
dangerous conditions which might result in loss  
of life or injury. To avoid this corrosion of the  
composite metal element, it has sometimes been  
customary in the past to treat the thermostatic  
metal surface to make it less subject to corrosion,  
as by plating it with a corrosion-resisting mate-  
rial, such as cadmium, tin, zinc, lead, or  
chromium. This, however, has the disadvantage  
that the plating increases the cost materially and  
does not assure satisfactory life for the thermo-  
static element. Furthermore, such plating is not  
entirely satisfactory since an electro-voltaic  
potential may be set up which produces pitting  
and eating away of the protective metal.

It has sometimes been the practice in the past

2

to make a composite metallic element from an  
iron alloy having a high chromium content, and  
a metal alloy having a higher coefficient of ex-  
pansion. The metal used for the high coefficient  
of expansion side has been one of the brasses.  
The mechanical properties of these brasses have  
presented manufacturing difficulties, which in  
many instances have prevented the manufacture  
of an adequate and satisfactory composite metal.  
10 For example, the cold-working properties of brass  
are so different from those of the chromium iron  
alloy that it has been difficult to satisfactorily  
cold-work the metal after it has been put to-  
gether to form a thermostatic bimetal. More-  
15 ever, it is highly advantageous in the manufac-  
ture of bimetal to hot-roll the material down  
from its thick ingot size to an intermediate stage.  
The brasses are not adapted to this, since their  
hot-rolling temperatures differ too much from  
20 that of the chromium iron alloy. The manufac-  
ture of the brass-chrome iron bimetals has there-  
fore been a relatively expensive process compared  
to the manufacture of bimetal in accordance with  
25 the present invention. The ingot size of the  
brass-chrome iron bimetals must be kept small  
because of the aforementioned difficulties and  
properties.

Where other constituents have been proposed  
30 for corrosion-resisting bimetals, it has been found  
relatively impossible to directly bond the metals  
together. For this reason, an intermediate solder  
layer has been used which has led to two serious  
35 disadvantages. First, the use of the solder layer  
decreases the corrosion-resisting property of the  
thermostatic metal due to inferior bonding, and  
second, the solder layer decreases the strength  
40 of the metal at elevated temperatures, since the  
solder bond is relatively weak. Also, solder-  
bonded material is difficult to hot-roll satisfac-  
torily.

By the present invention, it is possible to ac-  
complish a direct bond between the metals, and  
they may be hot-rolled or cold-rolled in the de-  
sired manner. Their manufacture is accordingly  
45 economical, and a highly corrosion-resisting  
thermostatic metal is obtained.

According to the present invention a thermo-  
static element is provided which is corrosion-  
50 resisting per se, particularly to air, water and  
water vapor, thus eliminating the need for sur-  
face plating. In addition, the present invention  
provides a thermostatic element made of com-  
posite thermostatic metal of the corrosion-resist-  
55 ing type which has a direct bond between the  
layers thereof.

The thermostatic metal of the present inven-

tion comprises layers of metal firmly secured together over their entire areas by a direct bond. One of the layers, in the present invention, comprises a corrosion-resisting metal having a low coefficient of expansion. The other layer comprises a second corrosion-resisting metal having a relatively high coefficient of expansion.

For the metal having a low coefficient of expansion a high chromium content stainless iron is employed. The composition of this alloy may 10 be as follows:

|           | Per cent  |
|-----------|-----------|
| Manganese | 0.2-0.6   |
| Carbon    | 0.01-0.2  |
| Chromium  | 12-20     |
| Silicon   | 0-1.5     |
| Copper    | 0-1.5     |
| Iron      | Remainder |

For the high expansion material an alloy of copper and silicon is employed. The composition of this alloy may be as follows:

|           | Per cent |
|-----------|----------|
| Copper    | 96-99    |
| Silicon   | 0.5-4    |
| Manganese | 0-1      |
| Tin       | 0-2.5    |

The composite thermostatic metal of which bimetal will be described as an illustrative embodiment may be formed in any of the customary manners. It is preferably formed in one of the ways described in my co-pending application, Serial No. 399,398, filed June 23, 1941, Patent 2,366,178, reference to which is hereby made.

Referring now to the drawing, the single figure illustrates a bimetallic element composed of the two alloys discussed above. Numeral 1 represents the copper silicon alloy while 3 is the iron chromium alloy.

The tensile strength and other mechanical properties of the copper silicon alloys described are sufficiently near to the same properties of the chrome-iron alloys that the two metals work well together and may be easily cold-worked. This makes the manufacture thereof more economical. As a result of obtaining a direct bond between the metals comprising the present invention, a thermostatic metal having a higher strength, greater activity, wider usable temperature range, longer life and better corrosion-resisting properties than the corrosion-resisting bimetals hitherto known, is obtained. Former metals allegedly designed to have these desirable properties have instead been relatively weak, corrode relatively easily, are more difficult to manufacture, and in general are not satisfactory.

As specific examples of alloys which may be advantageously employed in the present invention, the following examples are given. They are illustrative only:

#### Chrome-iron alloy

|           | Per cent |
|-----------|----------|
| Manganese | 0.4      |
| Carbon    | 0.05     |
| Chromium  | 16-20    |
| Iron      | Balance  |

#### Copper-silicon alloy No. 1

|         | Per cent |
|---------|----------|
| Copper  | 96-98    |
| Silicon | 2-4      |

#### Copper-silicon alloy No. 2

|         | Per cent |
|---------|----------|
| Copper  | 97       |
| Silicon | 3        |

Attention is directed to my copending applications, Serial Nos. 563,013, 563,014 and 563,016, all filed November 11, 1944.

In view of the above, it will be seen that the several objects of the invention are achieved and other advantageous results attained.

As many changes could be made in the above alloys without departing from the scope of the invention, it is intended that all matter contained in the above description shall be interpreted as illustrative and not in a limiting sense.

I claim:

1. A corrosion-resisting thermostatic metal of an alloy having essentially the following composition:

|           | Per cent |
|-----------|----------|
| Manganese | 0.4      |
| Carbon    | 0.05     |
| Chromium  | 16-20    |
| Iron      | Balance  |

and an alloy having essentially the following composition:

|         | Per cent |
|---------|----------|
| Copper  | 97       |
| Silicon | 3        |

the surfaces of said alloys being fused together at the junction.

30 2. A corrosion-resisting thermostatic metal composed of an iron alloy containing: manganese approximately 0.2-0.6%, carbon approximately 0.01-0.2%, chromium approximately 12-20%, and the balance iron; and a copper alloy containing: silicon approximately 0.5-4%, and the balance copper; the surfaces of said alloys being fused together at the junction.

35 3. A corrosion-resisting thermostatic metal composed of an alloy having essentially the following composition:

|           | Per cent |
|-----------|----------|
| Manganese | 0.4      |
| Carbon    | 0.05     |
| Chromium  | 16-20    |
| Iron      | Balance  |

45 and an alloy having essentially the following composition:

|         | Per cent |
|---------|----------|
| Copper  | 96-98    |
| Silicon | 2-4      |

50 the surfaces of said alloys being fused together at the junction.

4. A corrosion-resisting thermostatic metal composed of an alloy having essentially the following composition:

|           | Per cent |
|-----------|----------|
| Manganese | 0.2-0.6  |
| Carbon    | 0.01-0.2 |
| Chromium  | 12-20    |
| Iron      | Balance  |

60 and an alloy having essentially the following composition:

|         | Per cent |
|---------|----------|
| Copper  | 97       |
| Silicon | 3        |

the surfaces of said alloys being fused together at the junction.

55 5. A corrosion-resisting thermostatic metal composed of an alloy having essentially the following composition:

|           | Per cent |
|-----------|----------|
| Manganese | 0.2-0.6  |
| Carbon    | 0.01-0.2 |
| Chromium  | 12-20    |
| Iron      | Balance  |

and an alloy having essentially the following composition:

|         | Per cent |
|---------|----------|
| Copper  | 96-98    |
| Silicon | 2-4      |

the surfaces of said alloys being fused together at the junction.

PAUL G. CHACE.

REFERENCES CITED

The following references are of record in the file of this patent:

UNITED STATES PATENTS

| Number      | Name     | Date          |
|-------------|----------|---------------|
| 1,650,951   | Matthews | Nov. 29, 1927 |
| 1,929,655   | Scott    | Oct. 10, 1933 |
| 5 1,948,121 | Matthews | Feb. 20, 1934 |
| 1,991,438   | Wohrman  | Feb. 19, 1935 |
| 2,075,014   | Bassett  | Mar. 30, 1937 |

OTHER REFERENCES

10 Pp. 1000-1002 of The Making, Shaping, and Treating of Steel, 5th ed., 1940, pub. by Carnegie-Illinois Steel Corp., Pittsburgh, Pa.